

# United States Patent [19]

Seino et al.

[11] 3,812,565

[45] May 28, 1974

[54] **SINTERED FE—CR—C—[MO—V—NI]  
ALLOYS IMPREGNATED WITH PB OR  
RB-BASE ALLOYS**

[75] Inventors: **Hiroshi Seino, Yokohama; Shingichi  
Suzuno, Tokyo; Yoshiaki Takeya,  
Matsudo; Tsutomu Tobita, Matsudo;  
Takeshi Fukaya, Matsudo, all of  
Japan**

[73] Assignees: **Nissan Motor Company, Ltd.,  
Yokohama; Hitachi Powdered  
Metals Company, Matsudo, both of,  
Japan**

[22] Filed: **Dec. 19, 1972**

[21] Appl. No.: **316,545**

[30] **Foreign Application Priority Data**

Dec. 27, 1971 Japan..... 46-105526

[52] U.S. Cl. .... **29/182.1, 75/200**

[51] Int. Cl. .... **B22f 3/26, B22f 5/00, C22c 1/08**

[58] **Field of Search** ..... 29/182.1; 75/200; 252/12

[56] **References Cited**

UNITED STATES PATENTS

|           |         |                   |            |
|-----------|---------|-------------------|------------|
| 2,192,792 | 3/1940  | Kurtz .....       | 29/182.1 X |
| 2,409,307 | 10/1946 | Patch .....       | 29/182.1 X |
| 2,561,579 | 7/1951  | Lenel .....       | 29/182.1 X |
| 3,495,957 | 2/1970  | Matoba et al..... | 29/182.1   |

*Primary Examiner*—Leland A. Sebastian  
*Assistant Examiner*—R. E. Schafer

[57] **ABSTRACT**

A lead-filled sintered ferrous alloy containing carbon and chrome and preferably also molybdenum and vanadium is prepared in a powder metallurgy method and impregnated in its voids with lead. The alloy is characterized for its increased wear and heat resistant abilities and is accordingly advantageous when used as a material of a valve seat of an internal combustion engine using leadless fuel.

**9 Claims, 5 Drawing Figures**

PATENTED MAY 28 1974

3,812,565

SHEET 1 OF 3

Fig. 1



Fig. 2



PATENTED MAY 28 1974

3,812,565

SHEET 2 OF 3

Fig. 3



Fig. 4



PATENTED MAY 28 1974

3,812,565

SHEET 3 OF 3

*Fig. 5*



**SINTERED FE—CR—C—[MO—V—NI] ALLOYS  
IMPREGNATED WITH PB OR RB-BASE ALLOYS**

The present invention relates to sintered ferrous alloys and, more particularly, to sintered ferrous alloys having wear and heat resistant properties. In spite of the fact that the sintered ferrous alloy herein disclosed will find a wide variety of practical applications for wear resistant and high-temperature services, it will be described by way of example as specifically used as the material for valve seats for automotive internal combustion engines in which the valve seats are subject to serious wear and elevated temperature during operation.

Fuel containing lead or a lead compound such as tetraethyl lead as one of the typical chemical additives has long been employed for internal combustion engines of motor vehicles or other vehicles except for marine use. As is well known, the lead constituent in the automotive engine fuel is one of the major causes of vehicular air-pollution. To provide one solution to the problem, it is presently required to have such fuel supplanted by leadless fuel such as leadless gasoline and liquefied petroleum gas.

It is, however, pointed out that some barriers are encountered where the leadless fuel is combusted in the automotive engine. For one thing, the valve seat which is formed for instance of heat-resistant cast iron tends to be worn at its area to contact the valve face in a relatively short time to such an extent that the valve is no longer properly workable. A search for a material which is congruous for the valve seat of the internal combustion engine is thus currently subject of intensive research and development in the automotive and allied industries.

An object of the present invention is, therefore, to provide a new and useful material which is capable of withstanding wear and abrasion at elevated temperatures.

Another object of the invention is to provide a new and useful sintered ferrous alloy which is especially adapted for use as a material for a valve seat member of an automotive internal combustion engine.

Other objects and the nature and advantages of the sintered ferrous alloy provided in accordance with the present invention will become apparent from the following description of the invention when taken in conjunction with the accompanying drawing in which:

FIG. 1 is a graph indicating a relationship between tensile strength and temperature as exhibited in sintered ferrous alloys according to the present invention;

FIG. 2 is a graph indicating a relationship between tensile strength and temperature as exhibited in sintered ferrous alloys according to the present invention;

FIG. 3 is a graph illustrating variations in hardness against elevated temperature as observed in various metal materials including a sintered ferrous alloy proposed by the present invention;

FIG. 4 is a graph indicating a relationship between the coefficient of linear expansion and temperature in various sintered ferrous alloys including those implementing the present invention; and

FIG. 5 is a graph showing the amounts of wear in terms of time in hours of various metal materials including those which are provided in accordance with the present invention.

Two different materials appeared as usable for building the valve seat members of the internal combustion engines which are well compatible with leadless fuels — a sintered ferrous alloy having a lead constituent and a sintered ferrous alloy the voids of which are filled with lead.

According to the experiments we conducted, however, it has turned out that the ferrous alloy of the kind which is prepared by compacting and sintering metal particles in the presence of lead has a wear-resistant property which is short of the acceptable level. This is considered attributable to an insufficient mechanical strength of the base steel and to a limited proportion of the lead constituent in the ferrous alloy of the particular kind. The lead containing ferrous alloy produced in the powder metallurgy method is thus unacceptable as the material for the valve seat of the internal combustion engine using leadless fuel.

The sintered ferrous alloy filled with lead in its voids, on the other hand, has proved to have a wear resistance of an acceptable order, according to other experiments conducted by us. Bench tests were further conducted in which the valve seat formed of the lead filled ferrous alloy was actually installed on an automotive internal combustion engine. The sintered ferrous alloy used in these tests contained, on a weight basis, 3 percent of copper, 1.4 percent of molybdenum, 0.9 percent of carbon and the balance iron. The tests revealed that a considerable amount of play is invited between the valve seat member and the engine cylinder head in which the valve seat member was shrink fitted as usual. Although the particular material may find extensive and successful applications in general wear resistant services, the material is not acceptable as the wear and heat resistant material for the valve seat of the internal combustion engine.

Researches were therefore further conducted in quest for the reasons accounting for the fact that the lead impregnated sintered ferrous alloy fails to exhibit the expected mechanical properties when used in the internal combustion engines. Experiments were thus conducted with sintered ferrous alloys having and not having a lead filling therein for the purpose of examining the variation in tensile strength of these ferrous alloys at elevated temperatures, the results being demonstrated by curves *a* and *b* in FIG. 1. The curve *a* represents the sintered ferrous alloy filled with lead while the curve *b* represents the sintered ferrous alloy which is similar in composition to the former but which is void of the lead filling.

It is quite apparent from these curves *a* and *b* that the tensile strength of the lead filled ferrous alloy remains higher than that of the unfilled alloy within a temperature range from 50°C to about 200°C and diminishes steeply as the temperature rises beyond the particular range. The curves also indicate that, when the lead filled ferrous alloy is subjected to a temperature higher than the melting point of lead which is in the neighbourhood of 327°C as shown in FIG. 1, then the tensile strength of the alloy becomes outstandingly lower than that of the ferrous alloy not filled with lead. Though not shown, it was also ascertained that similar tendencies are exhibited in respect of the radial crushing strength of the alloys tested.

The valve seat member of the internal combustion engine usually has a limit in external size which is so prescribed that the seat member is interference or

shrink fitted into a mounting hole formed in the cylinder head. It therefore follows that the valve seat member is subjected to repeated expansion and contraction while being constantly under compression by the surrounding portion of the cylinder head, which is different from the sliding parts. In order that the valve seat member be will give satisfactory service in the engine cylinder, it should be endowed with not only a wear resistance of a sufficient order but also with an increased fatigue property against thermal shock. With this in mind, it is herein pointed out that the problems have thus far been involved in the prior art lead filled sintered ferrous alloys because of the fact that only those properties of the alloys which are displayed by the base steel which is to be filled with lead have been taken into consideration.

The goal of the present invention is, therefore, to provide an improved sintered ferrous alloy exhibiting sufficient wear resistance and fatigue property against thermal shock when used, for example, in the internal combustion engine using leadless fuel. Such goal has been achieved by virtue of intensive research and development covering a wide variety of sintered steels.

It was found in the course of the research and development programs that the hardness of a sintered ferrous alloy containing chrome and 0.6 to 1.2 percent by weight of carbon as alloying elements increases as the proportion of the chrome constituent increases and that the tensile strength of the alloy drops when the content of the chrome increases beyond 2.5 percent on a weight basis. This is graphically demonstrated in FIG. 2, in which the hardness of the alloy is indicated in terms of the diamond pyramid hardness number (DPH) under a 300-gram load. From FIG. 2, it is understood that both the hardness and tensile strength of the sintered ferrous alloy are acceptable where the alloy contains about 2 to 3 percent of chrome.

The present invention thus proposes a new lead filled sintered ferrous alloy containing 0.6 to 1.2 percent of carbon, 2 to 4 percent of chrome and the remaining percentage of iron on a weight basis. Experiments have revealed that the ferrous alloy having this composition is advantageous for use as a material for the valve seats of internal combustion engines which are driven under relatively light loads. For the valve seats to be incorporated in engines driven under heavier load conditions, it is preferable that the lead filled sintered ferrous alloys contain 0.6 to 1.2 per cent of carbon, 2 to 4 percent of chrome, 0.2 to 0.5 percent of molybdenum, 0.2 to 0.4 percent of vanadium and the remaining percentage of iron, all on a weight basis.

To add to the toughness of the lead-filled sintered ferrous alloy, the alloy may further contain 1 to 4 percent of nickel. This will prove advantageous where it is desired that the safety of operation of the engine be enhanced.

The lead with which the sintered ferrous alloy is filled may include not only elemental lead but also a lead based alloy having a relatively low melting temperature and containing at least one of tin, antimony, cadmium and bismuth. Where the sintered ferrous alloy according to the present invention is used as the material for the valve seats of internal combustion engines, the alloy filled with elemental lead will be suitable for engines driven at relatively high temperatures and the alloy filled with the lead alloy for engines driven at relatively low temperatures. Since, moreover, the proportion of the carbon in the alloy according to the present invention is limited to a range of 0.2 to 0.5 percent by weight, the mechanical strength of the alloy remains substantially constant irrespective of a change in the proportion of carbon. This will provide ease of controlling the sintering operation of the alloy and accordingly a stabilized quality of the final product.

The sintered ferrous alloy to be filled with lead is usually fabricated by the powder metallurgy method which in itself is well known in the art. In this instance, each of the constituents of the alloy may be provided in the form of powder of the element or, for the prevention of segregation of the particles and to provide ease of quality control, each constituent may be provided in the form of an alloy powder. The quantity of carbon, on the other hand, should be determined in consideration of the hydrogen loss.

Since, moreover, the ferrous alloy according to the present invention contains chrome, it is important that the mixed powders of the constituents be sintered in the presence of a highly reducing atmosphere with a relatively low humidity and at an elevated temperature.

The following table indicates compositions and mechanical properties of a representative prior art sintered ferrous alloy which is denoted by A and of the sintered ferrous alloys B, C and D which are prepared in accordance with the present invention. The prior art ferrous alloy A is prepared from mixed powders of elemental carbon, molybdenum, copper and iron and sintered at a temperature of 1,130°C for 30 minutes. The sintered ferrous alloys B and C according to the present invention are prepared each from a mixture of graphite powder and powders of alloying elements and sintered in an atmosphere of refined hydrogen at a temperature of 1,250°C for 30 minutes.

|                              | Known Alloy<br>A | Alloys of the Invention |         |         |
|------------------------------|------------------|-------------------------|---------|---------|
|                              |                  | B                       | C       | D       |
| Composition,<br>wt. %        |                  |                         |         |         |
| Carbon                       | 0.9              | 0.8                     | 0.8     | 0.8     |
| Chrome                       | Nil              | 3                       | 3       | 3       |
| Molybdenum                   | 1.4              | Nil                     | 0.4     | 0.4     |
| Vanadium                     | Nil              | Nil                     | 0.3     | 0.3     |
| Copper                       | 3                | Nil                     | Nil     | Nil     |
| Iron                         | Balance          | Balance                 | Balance | Balance |
| Density, g/cm <sup>3</sup>   | 6.8              | 6.8                     | 6.8     | 7.6     |
| Lead Filling, %              | Nil              | Nil                     | Nil     | 14      |
| Tensile Strength<br>at 300°C | Normal Temp. 42  | 72                      | 78      | 82      |
| at 500°C                     | 37               | 61                      | 71      | 77      |
| at 500°C                     | 28               | 55                      | 59      | 40      |
| Hardness Measure             | Normal Temp. 248 | 215                     | 260     | 60-70   |
|                              | 300°C 236        | 250                     | 287     | 60      |
|                              | 500°C 180        | 215                     | 226     | 57      |
|                              |                  | D P H                   |         | RHN     |

Continued

| Known Alloy                                        | Alloys of the Invention |       |       |
|----------------------------------------------------|-------------------------|-------|-------|
|                                                    | A                       | B     | C     |
| Young's Modulus, kg/mm <sup>2</sup>                | 12000                   | 12000 | 12000 |
| Limit of Elasticity, kg/mm <sup>2</sup>            | 45                      | 53    | 56    |
| Breaking Strength, kg/mm <sup>2</sup>              | 61                      | 62    | 67    |
| Coefficient of<br>200°C                            | 17.2                    | 11.5  | 11.3  |
| Linear Expansion<br>× 10 <sup>-6</sup> at<br>500°C | 14.6                    | 14.1  | 13.7  |
|                                                    |                         |       | 14.1  |

The sintered ferrous alloy B is an example in which only carbon and chrome are used as the alloying elements while the sintered ferrous alloy C is an example containing molybdenum and vanadium in addition to carbon and chrome as the alloying elements. The alloys A to C are all void of lead filling while the sintered ferrous alloy D is an example in which an alloy having the same composition as the alloy C has its pores filled with lead at a temperature of about 1,000°C. To ensure sufficient wear resistance property of the sintered ferrous alloy to be used as the material for the engine valve seats, it is important that the pores of the alloy be filled with at least 10 percent by weight of lead.

Comparison between the mechanical properties of the sintered ferrous alloys B and C according to the present invention will reveal that the mechanical properties are considerably improved through addition of molybdenum and vanadium as will be appreciated from the above presented table. It is, in this instance, preferable that the proportion of molybdenum is in the range of 0.2 to 0.5 percent by weight and the proportion of vanadium in the range of 0.2 to 0.4 percent by weight. Experiments have indicated that inclusion of these alloying elements in greater or smaller proportions than indicated results in impairment of the mechanical properties of the resultant ferrous alloy.

Tests were further conducted so as to examine the variation in hardness at elevated temperatures of the chrome containing, sintered ferrous alloy according to the present invention. The results of the tests on the alloy C having the composition indicated in the previously presented table are illustrated in FIG. 3 in comparison with these of the tests conducted on the prior art sintered ferrous alloy A and a heat-resistant cast iron of the composition complying with SAE D-3. The cast iron thus contains 2.2 percent of carbon, 0.35 percent of manganese, 2.6 percent of silicon, 3.4 percent of chrome, 1.0 percent of molybdenum and the remaining percentage of iron and impurities, all on a weight basis. From FIG. 3, it is quite apparent that the sintered ferrous alloy according to the present invention has peculiar properties as compared with the two prior art materials. While the hardnesses of the known sintered ferrous alloy and the specified heat-resistant cast iron diminish as they are subjected to rising temperatures, the sintered ferrous alloy C according to the present invention exhibits a property such that the hardness thereof increases as the temperature rises to the vicinity of 300°C. The hardness of the alloy C drops as the temperature rises beyond about 300°C but still remains at a level of the order of the hardness at a normal temperature when heated up to the vicinity of 400°C.

FIG. 4 illustrates curves indicating the variations of the coefficients of linear expansion at elevated temperatures of the sintered ferrous alloy A of the prior art composition and the sintered ferrous alloys C and D according to the present invention. These curves show that the coefficients of linear expansion of the ferrous alloys C and D are limited to relative low levels as com-

pared with that of the prior art ferrous alloy A. This means that, where the ferrous alloys C and D are used as the material for the valve seat members of the internal combustion engines, the valve seat members are subjected to significantly reduced expansion and contraction when the engine is being driven. The increased hardness and reduced variation in the coefficient of linear expansion at elevated temperatures of the material according to the present invention will thus considerably contribute to improvement of the heat-resistant ability and to prolongation of the service life of the valve seat members formed of such material.

For the purpose of rating the wear resistance of the valve seat member formed of the lead filled sintered ferrous alloy according to the present invention, bench tests were made on 1,800cc-capacity four-cylinder internal combustion engines using valve seats formed of the lead impregnated and unimpregnated sintered ferrous alloys D and C, respectively, and two known materials for the sake of comparison. The known materials were heat-resistant cast iron having the previously noted composition complying with SAE D-8 and heat-resistant steel complying with SAE HNV-6, viz., containing 0.80 percent of carbon, 0.40 percent of manganese, 2.30 percent of silicon, 20.00 percent of chrome, 1.30 percent of nickel and the remaining percentage of iron, on a weight basis. Every test was conducted for a continuous 100 hour period on a full-load basis, wherein the acceptance level was prescribed at 0.3 mm wear. The results of these bench tests are illustrated in FIG. 5. The satisfactory wear resistance character of the lead-impregnated sintered ferrous alloy according to the present invention can be ascertained from the curves illustrated in FIG. 5. A bench test was also conducted on a similar engine using valve seat members of a lead-filled sintered ferrous alloy having a composition similar to that of the sintered ferrous alloy B. The test revealed that the wear resistance of such material is somewhat inferior to, yet roughly comparable to that achieved by the sintered ferrous alloy C, though not shown in FIG. 5.

Tests were further made on motor vehicles in which the engine having valve seats of lead filled sintered ferrous alloy according to the present invention installed, and the vehicle driven a distance of 50,000 kilometers with use of liquefied petroleum gas. It was clearly ascertained that the lead filled sintered ferrous alloy according to the present invention is fully congruous for the valve seats of internal combustion engines using leadless fuel.

What is claimed is:

1. A wear and heat resistant composition comprising a sintered ferrous base alloy comprising 0.6 to 1.2 percent carbon by weight, 2 to 4 percent chromium by weight, and the remainder iron, the pores of said sintered ferrous base alloy being impregnated with a material selected from the group consisting of lead and lead based alloys, the material constituting at least 10 percent by weight of the ferrous base alloy.

2. A composition as claimed in claim 1 wherein said impregnated material is a lead based alloy containing at least one element selected from the group consisting of tin, antimony, cadmium and bismuth.

3. A composition as claimed in claim 1 wherein said impregnated material is lead.

4. A composition as claimed in claim 1 wherein said sintered ferrous base alloy further comprises 0.2 to 0.5 percent molybdenum by weight and 0.2 to 0.4 percent vanadium by weight.

5. A composition as claimed in claim 4 wherein said impregnated material is a lead based alloy containing at least one element selected from the group consisting

of tin, antimony, cadmium and bismuth.

6. A composition as claimed in claim 4 wherein said impregnated material is lead.

7. A composition as claimed in claim 4 wherein said sintered ferrous base alloy further comprises 1 to 4 percent nickel by weight.

8. A composition as claimed in claim 7 wherein said impregnated material is a lead based alloy containing at least one element selected from the group consisting of tin, antimony, cadmium and bismuth.

9. A composition as claimed in claim 7 wherein said impregnated material is lead.

\* \* \* \* \*